

## UNITED STATES PATENT OFFICE.

WILLOUGHBY STATHAM SMITH, OF NEWTON POPPLEFORD, AND HENRY JOSEPH GARNETT, OF SEVENOAKS, ENGLAND.

**MANUFACTURE OF WIRES AND TAPES FOR LOADING TELEPHONE CONDUCTORS.**

No Drawing. Application filed February 17, 1926, Serial No. 88,952, and in Great Britain February 17, 1925.

This invention relates to the manufacture of wires and tapes for loading telephone conductors.

According to this invention alloys suitable for the purpose are composed of nickel, copper and iron and free from carbon, in which the nickel ranges from 30% to 33% of the whole, the iron from 58% to 65% of the whole, and the copper from 2% to 6% of the whole.

As a result of our experiments we find that these alloys have valuable properties.

*Example.*

15 An alloy composed of:—

Per cent.

|        |    |
|--------|----|
| Nickel | 33 |
| Iron   | 65 |
| Copper | 2  |

20 has an initial permeability of 1000 and a specific resistance of 80 microms per cm<sup>3</sup>.

For certain purposes, such as for increasing the electrical resistance of the alloy, we introduced an additional element, which may be chromium, vanadium, tungsten, molybdenum, silicon, aluminum or titanium; the percentage of the added element should not exceed 3% while the combined percentage of the copper and the added element should not exceed 7%.

For example, an alloy prepared by us containing

Per cent.

|          |      |
|----------|------|
| Nickel   | 33   |
| Iron     | 64.5 |
| Copper   | 2    |
| Vanadium | 0.5  |

when suitably annealed had an initial permeability of 600 and a specific resistance of 85 microms per cm<sup>3</sup>.

When the vanadium is increased to 0.75% the specific resistance is 89 microms per cm<sup>3</sup> and the initial permeability 400.

An alloy of the following composition:—

|          | Per cent. |    |
|----------|-----------|----|
| Nickel   | 33        |    |
| Iron     | 63.5      |    |
| Copper   | 2.5       |    |
| Chromium | 1.0       | 50 |

gave an initial permeability of 610 and a specific resistance of 90 microms per cm<sup>3</sup>.

In order to develop the desired magnetic properties the alloys require suitable heat treatment. This consists of annealing in an atmosphere of nitrogen at a temperature of 850° to 930° C. followed by cooling in the same inert gas.

Small amounts of manganese not exceeding 1% may be added to promote forgeability and ductility.

What we claim is:—

1. Carbon free wires or tapes for loading magnetic conductors comprising nickel 30% to 33% of the whole, iron 58% to 65% of the whole, and copper 2% to 6% of the whole.

2. Carbon free wires or tapes for loading magnetic conductors comprising nickel 30% to 33% of the whole, iron 58% to 65% of the whole, copper 2% to 6% of the whole, and a fourth element not exceeding 3% of the whole and which is adapted to increase the electrical resistance, the combined percentage of the copper and said added element not exceeding 7% of the whole.

3. Carbon free wires or tapes for loading magnetic conductors comprising nickel 33% iron 63.5% copper 2.5%, and vanadium 0.5%.

In testimony that we claim the foregoing as our invention, we have signed our names this fifth day of February, 1926.

WILLOUGHBY STATHAM SMITH.  
HENRY JOSEPH GARNETT.